

UNITED STATES PATENT OFFICE

2,301,637

## ALUMINUM TANNING PROCESS

Joseph G. Niedercorn, Riverside, and William O. Dawson, Greenwich, Conn., assignors to American Cyanamid Company, New York, N. Y., a corporation of Delaware

**No Drawing. Application January 31, 1941,  
Serial No. 376,853**

**5 Claims. (Cl. 149—5)**

The present invention relates to the tanning of raw hides and skins and the like and has for its object to produce a white leather which is flexible and durable.

More specifically, this invention relates to the tanning of hides and skins with aluminum compounds and to a new aluminum tanning agent. It is well known that aluminum compounds may be used in the tanning of hides and skins.

The aluminum tanning agents of the prior art, such as alum, however, have proven unstable, and the tanning with aluminum compounds has been generally called "tawing" to distinguish it from a permanent tanning. The ability of aluminum compounds to produce a fine white leather has long been recognized and hence the desirability of the use of this compound as a tanning agent is well understood in the art. 10 15

We have found that a permanent white leather of good quality may be obtained by treating pickled hides and skins with the 100% basic aluminum salts of alpha-hydroxy isobutyric acid. The tanning with this compound may be carried out under neutral, alkaline, or slightly acid conditions. Our improved tanning agent may be used alone but is preferably used in conjunction with formaldehyde or by the various synthetic tanning agents.

The following example shows how our new tanning agent may be used in conjunction with formaldehyde.

### *Example*

100 pounds of skins having a pH of 1.5 were drummed for 15 minutes in a bath consisting of 12½ gallons of water containing 10 pounds of  $H_2SO_4$ . The pH of the liquor was 2.0. To this bath 10 pounds of formalin (37% HCHO) was added in three batches at 10 minute intervals and the skins were then drummed in the bath an additional 30 minutes. The pH of the liquor after the formalin addition was 2.1. Then 7 pounds of  $NaHCO_3$  dissolved in 6 gallons of water was added to the liquor in 6 batches at 15 minute intervals. The skins were drummed another two hours after which the skins were very plump and had a good feel. The pH of the liquor was 8.2, and the pH of the skins 7.6-7.8. The skins were then drained and washed for 15 minutes. The formaldehyde tanned skins were horsed up, set out and shaved. The skins were then put

back in the drum and to them was added gradually 50 pounds of a 40% aqueous solution of a 100% basic aluminum alpha-hydroxy isobutyrate followed by a further addition of 30 pounds of water. The skins were then drummed for 5 hours and left overnight in the liquor. The next day they were drummed an additional 30 minutes and then washed with water of gradually increasing temperature, from 100° F. to 125° F. The pH of the liquor before the skins were washed was 7.9, and the pH of the skins was 7.4-7.6. The skins had the same heat resistance after the aluminum tannage (89-90° C.) as after the formaldehyde tannage, the skins after the aluminum tannage were very white and had a good feel, although they fell slightly in the aluminum tannage. The skins were then fat liquored, horsed up overnight, and set out to dry. The skins, upon analysis, showed 72% hide substance, and 5.09% aluminum as aluminum oxide.

The 100% basic aluminum salt used in our new tanning process may be prepared by adding a water-soluble aluminum compound to an alpha-hydroxy isobutyric acid solution and then adding to the solution an alkaline compound of sodium or potassium, such as sodium hydroxide. Sufficient alkali must be added to neutralize the acid and to furnish an additional three moles of alkali metal per mole of aluminum present. The method of preparation of the basic aluminum salt of alpha-hydroxy isobutyrate is described more fully in our copending application, Serial No. 376,852, filed January 31, 1941. We believe that the basic aluminum salt has the following probable structural formula



where B stands for sodium or potassium.

In place of alpha-hydroxy isobutyric acid, its esters, such as ethyl alpha-hydroxy isobutyrate, may be saponified with sodium hydroxide, and used for the preparation of the aluminum salt in the same manner as the acid may be used. The complex aluminum salts may also be formed in situ, for example, by adding to the raw skins successively aluminum sulfate, sodium alpha-hydroxy isobutyrate and sodium bicarbonate.

Having now described our invention so that the same may be understood by those skilled in the art, what we claim is:

1. The improvement in the process of tanning hides and the like which consists in subjecting them to the action of a bath containing the 100% basic aluminum salt of alpha-hydroxy isobutyric acid.

2. The step in the process of tanning hides and the like which consists in subjecting the same to the action of a bath containing in solution a soluble aluminum compound, alpha-hydroxy isobutyric acid and an alkaline compound of sodium or potassium in excess of that required to neutralize the acid.

3. The improvement in the process of tanning hides and the like which comprises subjecting

them to the action of a bath containing a compound having the following structural formula



4. Leather tanned by the action of a water-soluble 100% basic salt of aluminum alpha-hydroxy isobutyrate.

5. Leather tanned by the action of a compound having the following structural formula.



JOSEPH G. NIEDERCORN.  
WILLIAM O. DAWSON.

CERTIFICATE OF CORRECTION.

Patent No. 2,301,637.

November 10, 1942.

JOSEPH G. NIEDERCORN, ET AL.

It is hereby certified that error appears in the above numbered patent requiring correction as follows: In the grant, line 4, and in the heading to the printed specification, line 6, state of incorporation of the assignee, for "Delaware" read --Maine--; and that the said Letters Patent should be read with this correction therein that the same may conform to the record of the case in the Patent Office.

Signed and sealed this 22nd day of December, A. D. 1942.

(Seal)

Henry Van Arsdale,  
Acting Commissioner of Patents.